

## UNITED STATES PATENT OFFICE

2,654,146

## GOLD BASE ALLOY

Victor G. Mooradian, East Orange, N. J., assignor  
to The H. A. Wilson Company, Newark, N. J.,  
a corporation of New Jersey

No Drawing. Application April 2, 1949,  
Serial No. 85,261

12 Claims. (Cl. 29—199)

**1** This invention relates to gold-base alloys, and more particularly to gold-base alloys containing silicon together with iron, chromium or zirconium for the jewelry trade.

Gold-base alloys heretofore commonly used for making jewelry articles frequently develop the defect known as "orange peel" when the alloy is alternately subjected to annealing at a high temperature and severe mechanical working at room temperature. This defect is characterized by a surface roughness similar in appearance to the outer surface of the skin of an orange (though on a finer scale), whence comes the name "orange peel." It is objectionable because a great deal of polishing is necessary to restore a smooth surface to the article on which it develops. It is particularly objectionable when it develops on the gold alloy cladding layer of rolled gold plate, because this thin layer is often polished completely through in the effort to obliterate the orange peel roughness.

The gold alloys subject to development of orange peel roughness are mostly the standard 10-karat to 18-karat alloys containing about 1% to 55% copper, 1% to 15% silver, 1% to 15% zinc, sometimes a fraction of 1% to 4% nickel, and the balance gold. (All percentages herein are by weight.) I have discovered that by the addition to such alloys of 0.01% to 1% silicon together with 0.1% to 3% of a metal selected from the group consisting of iron, chromium, and zirconium, the tendency for orange peel to develop is substantially inhibited. It is, moreover, inhibited permanently. For example, the standard alloys described above may not display any tendency to develop objectionable orange peel roughness when first annealed or when first worked, but may develop this defect rather suddenly after being subjected to two or more successive working operations with intermediate anneals. When silicon together with iron, chromium or zirconium is incorporated in the alloy in the amount stated, no substantial orange peel roughness develops regardless of the number of alternate anneals and working operations to which the alloy is subjected.

Especially satisfactory results have been obtained by the addition of from 0.05% to 0.5% silicon and from 0.5% to 1.5% iron, chromium or zirconium to a 10-karat to 14-karat yellow gold alloy of 25% to 50% copper, 3% to 10% silver, 3% to 10% zinc, from none up to 2% of nickel, and the balance (usually about 40% to 60%) gold. For example, a 10-karat alloy consisting of 41.6% gold, 42.0% copper, 7.1% silver, 8.2% zinc and

1.1% nickel always displays a marked orange peel surface condition when a sheet of such material is subjected to a treatment involving annealing to the dead soft condition, then cold rolling to the extent of 50% reduction in area, then annealing for 15 minutes at 1300° F., and then drawing to the breaking point with a round-bottom punch in a bottomless die. By incorporating 0.1% silicon and 1.0% iron, chromium or zirconium in this particular alloy (proportionately reducing the amounts of copper, silver and zinc), the tendency for it to develop orange peel is quite completely inhibited, both when it is given the same treatment just described and when given the even more severe treatment involving increasing the final annealing temperature from 1300° F. to 1600° F.

The gold alloys of the invention are easily fabricated into rolled gold plate by the customary procedure of bonding a layer of the new alloy to a bar of base metal and then rolling the composite bar to the desired final thickness. The provision of such composite metal products is an especially advantageous feature of the invention, because the new gold-base alloy is able to withstand the high annealing temperatures to which the base metal often must be subjected, without developing orange peel roughness. The base metals used in the fabrication of rolled gold plate (such, for example, as commercial "L" nickel, or "composition metal"—sometimes called "gilding metal"—which is basically a low-zinc brass, or a nickel silver alloy composed of about 45% to 60% copper, about 10% to 30% nickel, about 15% to 25% zinc, and sometimes a few per cent of tin and lead) have annealing temperatures upwards of 1000° F., and often must be heated to such temperature or higher in the course of being fabricated by cold working into intricate jewelry articles. The standard karat gold alloys easily develop orange peel roughness when subjected to severe mechanical working after having been heated to the base metal annealing temperature above 1000° F., and particularly above 1200° F. Consequently, rolled gold plate made by bonding a standard karat gold alloy to a base metal having an annealing temperature above 1000° F. cannot be heated to the full annealing temperature of the base metal and then worked without developing orange peel roughness. Since the thickness of the gold layer on the finished plate is generally only a few thousandths of an inch, it is particularly undesirable to have orange peel develop on this very thin layer when it is fabricated into a watchcase

or other jewelry item. Polishing the thin gold alloy layer at those points where orange peel roughness develops frequently results in wearing completely through the gold alloy layer. However, a composite metal product comprising a sheet of base metal having an annealing temperature upwards of 1000° F. to which is bonded a surface layer or sheet of a gold-base alloy containing silicon together with iron, chromium or zirconium in accordance with the invention may be heated to the full annealing temperature of the base metal without having orange peel roughness develop to any significant extent at the surface of the gold alloy layer when the composite product is thereafter subjected to severe plastic deformation.

The inclusion of silicon together with iron, chromium, or zirconium has no detrimental effect on the corrosion resistance of the alloy, and may even improve it somewhat. Further, these alloys are precipitation hardenable by the process of heating to a temperature of about 1200° to 1300° F., quenching to room temperature, and then re-heating at about 550° to 700° F. for about two hours. Advantage may be taken of this property in the fabrication of jewelry items in which rather high strength and hardness are desirable.

I claim:

1. A composite metal product comprising a sheet of base metal having an annealing temperature upwards of 1200° F. to which is bonded a surface layer a few thousandths of an inch in thickness of an alloy consisting essentially of 1% to 55% copper, 1% to 15% silver, 1% to 15% zinc, 0.01% to 1% silicon, 0.1% to 3% of a metal selected from the group consisting of iron, chromium, and zirconium, and the balance gold, whereby said composite metal may be alternately heated to above the annealing temperature of its base metal component and subjected to severe mechanical working at room temperature without developing significant orange peel roughness at the surface of the gold alloy layer.

2. A composite metal product comprising a sheet of base metal having an annealing temperature upwards of 1200° F. to which is bonded a surface layer a few thousandths of an inch in thickness of an alloy consisting essentially of 1% to 55% copper, 1% to 15% silver, 1% to 15% zinc, 0.01% to 1% silicon, 0.1% to 3% iron, and the balance gold, whereby said composite metal may be alternately heated to above the annealing temperature of its base metal component and subjected to severe mechanical working at room temperature without developing significant orange roughness at the surface of the gold alloy layer.

3. A composite metal product comprising a sheet of base metal having an annealing temperature upwards of 1200° F. to which is bonded a surface layer a few thousandths of an inch in thickness of an alloy consisting essentially of 1% to 55% copper, 1% to 15% silver, 1% to 15% zinc, 0.01% to 1% silicon, 0.1% to 3%

chromium, and the balance gold, whereby said composite metal may be alternately heated to above the annealing temperature of its base metal component and subjected to severe mechanical working at room temperature without developing significant orange peel roughness at the surface of the gold alloy layer.

5. A composite metal product comprising a sheet of base metal having an annealing temperature upwards of 1200° F. to which is bonded a surface layer a few thousandths of an inch in thickness of an alloy consisting essentially of 1% to 55% copper, 1% to 15% silver, 1% to 15% zinc, 0.01% to 1% silicon, 0.1% to 3% zirconium, and the balance gold, whereby said composite metal may be alternately heated to above the annealing temperature of its base metal component and subjected to severe mechanical working at room temperature without developing significant orange peel roughness at the surface of the gold alloy layer.

6. An alloy having increased resistance to the development of orange peel when ultimately subjected to annealing at high temperature and severe mechanical working at room temperature consisting essentially of from about 1% to 55% copper, from about 1% to 15% silver, from about 1% to 15% zinc, from about 0.01% to 1% silicon, from about 0.1% to 1.5% of a metal selected from the group consisting of iron, chromium and zirconium, and the balance gold.

7. An alloy as defined in claim 5 in which the metal of said group is iron.

8. An alloy as defined in claim 5 in which the metal of said group is chromium.

9. An alloy as defined in claim 5 in which the amount of copper is from about 25% to 50%.

10. An alloy as defined in claim 5 in which the amount of silver is from about 3% to 10%.

11. An alloy as defined in claim 5 in which the amount of zinc is from about 3% to 10%.

12. An alloy as defined in claim 5 which contains nickel in amount up to about 2%.

VICTOR G. MOORADIAN.

References Cited in the file of this patent

UNITED STATES PATENTS

| Number       | Name     | Date          |
|--------------|----------|---------------|
| 1,571,540    | Davignon | Feb. 2, 1926  |
| 1,580,444    | Shields  | Apr. 13, 1926 |
| 55 1,725,445 | Davignon | Aug. 20, 1929 |
| 1,712,244    | Bek      | May 7, 1929   |
| 2,007,008    | Staples  | July 2, 1935  |
| 2,141,157    | Peterson | Dec. 29, 1938 |
| 2,248,100    | Loebich  | July 8, 1941  |
| 60 2,229,463 | Leach    | Jan. 21, 1941 |
| 2,270,594    | Leuser   | Jan. 20, 1942 |
| 2,394,673    | Edmonds  | Feb. 12, 1946 |

FOREIGN PATENTS

| Number     | Country     | Date          |
|------------|-------------|---------------|
| 65 218,138 | Switzerland | Mar. 16, 1942 |